

## 1

3,301,782

## ADDUCTS OF ZINC COMPOUNDS AND LUBRICANTS CONTAINING SAME

Edwin C. Knowles, Poughkeepsie, and Frederic C. McCoy, Beacon, N.Y., assignors to Texaco Inc., New York, N.Y., a corporation of Delaware  
No Drawing. Filed Oct. 9, 1963, Ser. No. 314,886  
13 Claims. (Cl. 252—46.4)

The present invention relates to novel adducts of zinc compounds and to a lubricating composition comprising a lubricating oil and an adduct of an amine or Schiff base and a zinc compound.

New designs and improvements in machinery are continually raising the operating performance standards of lubricating oil compositions. In many instances, the pressures and temperatures under which the bearing surfaces of machinery operate are higher than those which natural or synthetic lubricating oils can withstand. Difficult lubricating conditions are commonly encountered in the lubrication of heavily loaded pinion and spur gears, gear trains, bearings, extrusion applications and the like. As a result, there is an increasing need for lubricating compositions having improved properties for these services.

A novel class of oil-soluble amine or Schiff base adducts of zinc compounds has been discovered which imparts greatly improved properties to lubricating oils. The lubricant compositions containing the adducts are particularly notable for their improvement in load carrying and anti-scuff properties although they also exhibit additional advantages in corrosion resistance, oxidation resistance and stability. These lubricating compositions provide the answer to some heretofore difficult lubrication problems.

The novel oil-soluble adduct of the invention is formed from the reaction of an amine or a Schiff base and zinc silicofluoride, phosphate, hypophosphite, sulfite or thiocyanate. More particularly, the adduct of the invention is represented by one of the following formulas:

(a)  $(RR'N)_xX$   
and

(b)  $(R''N=CR')_yX$

in which R is a hydrocarbyl radical having from 6 to 30 carbon atoms, R' is selected from the group consisting of hydrogen and a hydrocarbyl radical having from 1 to 30 carbon atoms, R'' is an aliphatic radical having from 1 to 30 carbon atoms, the sum of the carbon atoms in either of the compounds represented by (a) and (b) being at least 12, y is an integer from 1 to 6 and X is a zinc compound selected from the group consisting of zinc silicofluoride, zinc phosphite, zinc hypophosphite, zinc sulfite and zinc thiocyanate.

Amines which can be employed to prepare the adduct of the invention are the amines having one or more hydrocarbyl radicals in which the total number of carbon atoms in said amine is at least 12. The requirement of 12 carbon atoms in the amine is critical to insure the oil solubility of the adduct. Adducts formed from amines having less than 12 carbon atoms are generally not soluble in lubricating oils. The effective amines correspond to the formula:

$RR'_2N$

wherein R is a hydrocarbyl radical having from 6 to 30 carbon atoms and R' is hydrogen or a hydrocarbyl radical having from 1 to 30 carbon atoms. R is generally a branched chain alkyl radical because of the ready availability of these materials. Preferably, R is a tertiary alkyl radical having from 12 to 30 carbon atoms. R may, however, be an aryl, aralkyl or alkaryl radical having the prescribed number of carbon atoms. R' repre-

## 2

sents hydrogen or a hydrocarbyl radical having from 1 to 30 carbon atoms of the same types defined for R.

Examples of effective amines include laurylamine, tridecylamine, tetradecylamine, hexadecylamine, octadecylamine, eicosylamine, tricosylamine, nonacosylamine, nonylphenylamine, dodecylphenylamine, methyldodecylamine, dimethyldodecylamine, methyloctadecylamine, and dimethyloctadecylamine. Particularly preferred amines are certain commercially available mixtures of tertiary alkyl primary amines. For example, a mixture of tertiary alkyl primary amines in which the alkyl radical comprises a mixture of alkyl groups having from 11 to 14 carbon atoms is available under the name Primene 81-R. Another commercially available amine is the mixture of tertiary alkyl primary amines in which the alkyl radical comprises a mixture of alkyl groups having 18 to 24 carbon atoms sold under the name Primene JM-T.

The Schiff base which corresponds to the formula:



in which R' and R'' have the values noted above and which is employed to form the adduct of the invention is prepared from an amine and an aldehyde. Specifically, equivalent amounts of a primary amine and an aldehyde are contacted either in the presence of or without a solvent. The reaction frequently occurs spontaneously although at times moderate heating is required. A mole of water splits out in the formation reaction of the Schiff base. The water formed by the reaction is generally removed by azeotroping with a solvent, such as toluene. It is essential that the sum of the carbon atoms represented by R' and R'' in the formula for the Schiff base amount to at least 12 in order to insure the oil solubility of the adduct that is to be formed.

Amines which can be employed to prepare the Schiff base are the primary aliphatic amines. These amines are represented by the following formula:



in which R is an aliphatic hydrocarbyl radical having from 1 to 30 carbon atoms. The preferred amines are those in which R is a branched chain alkyl radical having from about 12 to 24 carbon atoms.

Examples of suitable primary amines for the Schiff base reaction include butylamine, amylamine, hexylamine, octylamine, laurylamine, tridecylamine, tetradecylamine, hexadecylamine, octadecylamine, and tricosylamine and the above defined Primene 81-R and Primene JM-T.

Aldehydes which can be employed to react with the above described primary amines to form the Schiff base are represented by the following formula:



in which R' is hydrogen or a hydrocarbyl radical having from 1 to 30 carbon atoms. The hydrocarbyl radical can be an aliphatic or an aromatic hydrocarbyl radical and preferably has from 1 to 10 carbon atoms. Examples of effective aldehydes for this reaction include formaldehyde, 2-ethylhexaldehyde, acetaldehyde, propionaldehyde, butyraldehyde, nonylaldehyde, palmitaldehyde, lauraldehyde, stearaldehyde, benzaldehyde and salicylaldehyde.

The adducts of the invention are prepared by mixing from 1 to 6 moles, preferably 1 to 4 moles, of a hydrocarbyl amine or a Schiff base defined above with a mole of zinc silicofluoride, zinc phosphite, zinc hypophosphite, zinc sulfite or zinc thiocyanate. This reaction is usually exothermic and provision must generally be made to cool the reaction mixture. In particular, caution must be exercised to keep the reaction temperature below the decomposition temperature of the various components of the

reaction product or adduct which generally means conducting the reaction at a temperature below about 200° C. The reaction generally goes to completion in a short reaction time.

The reaction of a zinc compound with an amine or a Schiff base to form the adduct of the invention is unpredictable. Many zinc compounds do not form adducts with either the amines or Schiff bases. For example, zinc fluoride, zinc borate, zinc sulfate, zinc sulfide and zinc oxide would not form adducts with the amines or Schiff bases.

Examples of adducts of the invention are given below. For convenience, the Schiff base part of the adducts listed is expressed in terms of the components from which the Schiff bases are formed. The mole ratio in parenthesis is the ratio of the amine or Schiff base to the zinc compound.

Primene JM-T:zinc sulfite (4:1)  
 Primene JM-T:zinc phosphite (2:1)  
 Primene JM-T:zinc phosphite (1:1)  
 Primene JM-T:zinc silicofluoride (2:1)  
 Primene JM-T:zinc thiocyanate (2:1)  
 Primene JM-T:zinc hypophosphite (3:1)  
 Primene 81-R:zinc silicofluoride (2:1)  
 Primene 81-R:zinc thiocyanate (2:1)  
 Primene JM-T/formaldehyde:zinc phosphite (2:1)  
 Primene JM-T/2-ethylhexaldehyde:zinc thiocyanate (2:1), and  
 Primene JM-T/2-ethylhexaldehyde:zinc silicofluoride (3:1).

The lubricating composition of the invention is prepared by blending in a conventional way a minor amount of the oil-soluble, load-carrying hydrocarbyl amine or Schiff base-zinc compound adduct described hereinabove into a suitable lubricating oil base. Generally, the adduct is employed in an amount in the range of 0.05 to 10 percent by weight based on the weight of the lubricating composition with the preferred proportions of the adduct being from 0.1 to 3 weight percent.

The base lubricating oil can be a mineral lubricating oil or a synthetic lubricating oil. The mineral lubricating oil can be a predominantly paraffinic or naphthenic oil or can be a mixture of the two types of mineral oils. Generally, the mineral oil will be a refined oil of predominantly paraffinic nature, having a viscosity in the range from 30 to 150 Saybolt Universal seconds at 210° F.

Various types of synthetic lubricating oil bases can be employed in preparing the lubricants of the invention. Aliphatic ester, polyalkylene oxides, silicones, esters of phosphoric and salicylic acid and the highly fluorine-substituted hydrocarbons can be employed. Examples of the aliphatic esters include di-(2-ethylhexyl) sebacate, the dialkyl azelates, dialkyl suberates, and the dialkyl adipates such as di-hexyl azelate, di-(2-ethylhexyl) azelate, di-3,5,5-trimethylhexyl gluterate, di-(2-ethylhexyl) adipate, triamyl tricarboxylate, etc. The polyalkylene oxide lubricants include polyisobutyloxide, polyisopropylene oxide diether, polyisopropylene oxide diesters, etc. The silicone lubricants include methyl silicone, methylphenyl silicone and the silicate lubricants include tetraisoctyl silicate. The highly fluorinated hydrocarbon lubricants include

fluorinated oil, perfluorohydrocarbons and the like.

Other effective synthetic lubricating oils include the neopentyl glycol esters such as the neopentyl glycol propionates, neopentyl glycol butyrate and the neopentyl glycol caprylates and the trimethylol alkanes such as trimethylethane, trimethylol propane, trimethylol pentane, trimethylol heptane and trimethylol dodecane and the like. Examples of the phosphate esters include tricresyl phosphate, trioctyl phosphate and tridecyl phosphate as well as mixed aryl and alkyl phosphates.

#### Example I

The load carrying and anti-scuff properties of lubricating compositions of the invention were determined in a number of standard tests. The Mean Hertz Load Test is run in a machine having four 1/2 inch diameter bearing balls which are driven under load while being lubricated by the composition under test. The description of this test is set forth in U.S. Patent 2,600,058.

In the Ryder Gear Test (Federal Test Method 6508), the lubricant being tested is employed to lubricate two spur gears in a Pratt and Whitney Gear and Lubricating Tester. This tester was operated with a gear speed of 10,000 r.p.m. and with an oil inlet temperature of 165° F. The loading pressure of 5.0 p.s.i. was applied during break-in. After 10 minutes the tester was shut down and the gear examined for the percentage of tooth area scuff on each tooth. This procedure was repeated using a high load pressure with increments of 5 p.s.i. until 22.5 percent of the total tooth area on the driving gear had been scuffed, the load applied in this run being considered the scuff load. The tooth load in pounds per inch of tooth width was then calculated.

The Navy Four Ball Wear Test also measures the anti-wear properties of a lubricant. The test machine employed comprises a system of four steel balls, three of which are in contact with each other in one plane in a fixed triangular position in a reservoir containing the oil sample and a fourth ball is above and in contact with the other three. In carrying out the test, the upper ball is rotated at a speed of 1800 r.p.m while it is pressed against the lower three at a constant load of 28 kg. for four separate periods of 10, 40, 70 and 100 minutes. The wear rate is calculated in microns per minutes.

The Mean Hertz Load was determined by means of the same equipment used in the Navy Four Ball Wear Test, using Federal Test Method Standard 791A, Method 6503.

Lubricating compositions illustrative of the invention were prepared from both mineral and synthetic lubricating oils. The mineral lubricating oil was essentially a paraffinic lubricating oil having an SUS viscosity at 210° F. of about 100. This is designated as Base Oil A. The synthetic lubricating oil consisted of di-2-ethylhexyl sebacate plus sebacic acid. This oil, which is commercially available as Plexol 201J, is designated as Base Oil B in the example. The adduct mole ratio indicated in parenthesis is the mole ratio of the hydrocarbylamine or of the Schiff base employed to the zinc compound. Schiff Base A was formed by reacting a mole of Primene JM-T with a mole of 2-ethylhexaldehyde. The test results are given in Table I below.

TABLE I.—LOAD CARRYING AND ANTI-SCUFF PROPERTIES

| Adduct (Mole Ratio)                        | Percent By Wt. | Base Oil | Ryder Gear Test, p.p.i. | Mean Hertz Load | Navy Four Ball Wear Test, micron/min. |
|--------------------------------------------|----------------|----------|-------------------------|-----------------|---------------------------------------|
| None                                       |                |          |                         |                 |                                       |
| Primene JM-T/ZnHPO <sub>4</sub> (3:1)      | 1.0            | A        | 2,300                   | 16              | 11.8, 8.7                             |
| Primene JM-T/ZnSiF <sub>6</sub> (2:1)      | 1.0            | A        | 4,320                   | -----           | 0.2                                   |
| Primene JM-T/ZnSiF <sub>6</sub> (2:1)      | 2.0            | A        | -----                   | 49              | -----                                 |
| Schiff's Base A/ZnHPO <sub>4</sub> (4:1)   | 1.0            | A        | -----                   | 26              | 0.6                                   |
| Schiff's Base A/Zn(SCN) <sub>2</sub> (2:1) | 1.0            | A        | -----                   | 28              | 1.8                                   |
| Primene JM-T/Zn(SCN) <sub>2</sub> (2:1)    | 1.0            | A        | -----                   | 24              | -----                                 |
| Primene JM-T/ZnSO <sub>4</sub> (4:1)       | 1.0            | -----    | -----                   | 32              | 8.2                                   |
| Primene JM-T/ZnHPO <sub>4</sub> (2:1)      | 0.5            | A        | -----                   | -----           | 0.9                                   |
| None                                       |                | B        |                         | 18              | -----                                 |
| Primene JM-T/ZnSiF <sub>6</sub> (2:3)      | 1.0            | B        | -----                   | 24              | -----                                 |

The lubricating compositions containing the above-described amine or Schiff base-zinc compound adducts have markedly improved load-carrying, wear and anti-scuff properties. They also exhibit good corrosion resistance, oxidation resistance and storage stability. These valuable properties make the lubricants of the invention suitable for a broad range of lubrication applications.

It is understood that the lubricating compositions of the invention can contain numerous additives conventionally used to improve the properties of lubricating oils. Commonly employed additives are the methacrylates as V.I. improvers and pour point depressors, the alkylphenols as oxidation inhibitors, alkaline earth metal salts of petroleum sulfonates or alkaryl sulfonates as detergents, metal dialkyl dithiophosphate corrosion inhibitors and silicone anti-foam fluids.

Obviously, many modifications and variations of the invention as hereinbefore set forth may be made without departing from the spirit and scope thereof and, therefore, only such limitations should be imposed as are indicated in the appended claims.

We claim:

1. A novel composition produced by reacting 1 to 6 moles of a compound represented by a formula selected from the group consisting of:



in which R is an alkyl radical having from 6 to 30 carbon atoms, R' is selected from the group consisting of a hydrogen and an alkyl radical having from 1 to 30 carbon atoms and R'' is an alkyl radical having from 1 to 30 carbon atoms, the sum of the carbon atoms in the compound represented by (a) and (b) being at least 12, with a mole of a zinc compound selected from the group consisting of zinc silicofluoride, zinc phosphite, zinc hypophosphite, zinc sulfite and zinc thiocyanate.

2. A composition according to claim 1 in which said zinc compound is zinc silicofluoride.

3. A composition according to claim 1 in which said zinc compound is zinc phosphite.

4. A composition according to claim 1 in which said zinc compound is zinc hypophosphite.

5. A composition according to claim 1 in which said zinc compound is zinc sulfite.

6. A composition according to claim 1 in which said zinc compound is zinc thiocyanate.

7. As a new composition, the product produced by reacting 4 moles of a  $C_{18-24}$  alkyl primary amine with a mole of zinc silicofluoride.

8. As a new composition, the product produced by reacting 4 moles of a Schiff base with a mole of zinc phos-

phite, said Schiff base being obtained by reacting a mole of a  $C_{18-24}$  alkyl primary amine with a mole of 2-ethylhexaldehyde.

9. As a new composition, the product produced by reacting 2 moles of a Schiff base with a mole of zinc thiocyanate, said Schiff base being obtained by reacting a mole of a  $C_{18-24}$  alkyl primary amine with a mole of 2-ethylhexaldehyde.

10. A lubricating composition comprising a major proportion of a lubricating oil and 0.05 to 10 percent by weight of an oil-soluble composition produced by reacting 1 to 6 moles of a compound represented by a formula selected from the group consisting of:

15 (a)  $RR'_2N$   
and  
(b)  $R''N=\overset{H}{\underset{R'}{C}}$   
20 in which R is an alkyl radical having from 6 to 30 carbon atoms, R' is selected from the group consisting of hydrogen and an alkyl radical having from 1 to 30 carbon atoms and R'' is an alkyl radical having from 1 to 30 carbon atoms, the sum of the carbon atoms in the compound represented by (a) and (b) being at least 12, with a mole of a zinc compound selected from the group consisting of zinc silicofluoride, zinc phosphite, zinc hypophosphite, zinc sulfite and zinc thiocyanate.

25 11. A lubricating composition according to claim 10 in which said oil-soluble compound is the product produced by reacting 4 moles of a  $C_{18-24}$  alkyl primary amine with a mole of zinc silicofluoride.

30 12. A lubricating composition according to claim 10 in which said oil-soluble compound is the product produced by reacting 4 moles of a Schiff base with a mole of zinc phosphite, said Schiff base being obtained by reacting a mole of a  $C_{18-24}$  alkyl primary amine with a mole of 2-ethylhexaldehyde.

35 13. A lubricating composition according to claim 10 in which said oil-soluble compound is the product produced by reacting 2 moles of a Schiff base with a mole of zinc thiocyanate, said Schiff base being obtained by reacting a mole of a  $C_{18-24}$  alkyl primary amine with a mole of 2-ethylhexaldehyde.

#### References Cited by the Examiner

##### UNITED STATES PATENTS

|    |           |         |              |           |
|----|-----------|---------|--------------|-----------|
| 50 | 2,112,567 | 3/1938  | Havas        | 260—429.9 |
|    | 2,725,358 | 11/1955 | Kluge et al. | 252—42.7  |
|    | 3,107,739 | 10/1963 | Mathews      | 260—429.9 |

DANIEL E. WYMAN, Primary Examiner.

55 L. G. XIARHOS, Assistant Examiner.